

## 1

2,938,811

**METHOD OF CONDITIONING POLYESTER TEXTILE MATERIAL AND THE RESULTING PRODUCTS**

Julius Hermes, Martinsville, Va., assignor to Martin Processing Company, Incorporated, Martinsville, Va., a corporation of Virginia

No Drawing. Filed Nov. 9, 1959, Ser. No. 851,506

5 Claims. (Cl. 117—102)

This invention relates to the treatment of synthetic textile material of the kind known as "Dacron" which, as is well known in the art, is a condensation polymer of terephthalic acid and ethylene glycol, also known as polyethylene terephthalate or, perhaps more familiarly, as polyester material. More particularly, the invention relates to a procedure for conditioning such material whereby it is given substantially new and different properties rendering it especially adaptable to subsequent processing. The invention also relates to the resulting products, and especially to the undyed products resulting from the conditioning treatment. Reference to synthetic textile material or polyester material hereinafter is to be regarded for the sake of brevity as referring solely to the aforesaid synthetic textile material unless indicated otherwise by the context.

The method of this invention comprises subjecting the polyester material to heating at a very high temperature using a hot liquid medium for effecting the heating. The importance of this type of heating is the liquid or wet, as distinguished from the conventional dry form of heating, such as on drying cans or the like. The liquid heat treatment effects an actual impregnation of the polyester textile material with the hot liquid that imparts to the treated material new properties, e.g. anti-pilling properties, not obtainable by dry heating, and likewise conditions the polyester material for more effective additional treatments such as, for example, dyeing. This liquid heat treatment or conditioning of the polyester material is preferably carried out without supplemental treatment thereof except for removal or substantial removal of the heating liquid. Alternatively, this liquid heat treatment may be carried out first and then followed by additional treatments of the polyester material such as dyeing, since the polyester material is thereby rendered especially amenable to dyeing.

This subsequent treatment of the polyester textile material, however, is not required and is used only when and as desired to produce some additional characteristic, such as, for example, dyeing of the material. Independently of dyeing or other subsequent operation, the polyester material treated with the highly heated liquid in accordance with the present invention acquires new physical properties, such as the above mentioned anti-pilling property.

The anti-pilling property is especially important. It has been found that fabrics or garments made from the foregoing polyester textile fibers or mixtures thereof with other fibers, when subjected to abrasion such as is ordinarily encountered in wearing or laundering, will produce "pills" or small balls of the abraded fibers that do not fall off or become separated from the fabric, but adhere to it and produce a very unattractive surface appearance. This effect is in contrast to the abrasion effects experienced with wool and other natural fibers, and in which pills or balls either do not form on the surface of the goods or if they do form they break off, leaving a smooth uni-

## 2

form surface. It appears that the pills or balls formed on the polyester fiber materials do not break or fall off because of the increased strength and perhaps other characteristics of these fibers different from the natural fibers.

This pilling problem has become acute in view of the fact that the polyester fiber fabrics and garments of the kind mentioned above exhibit this undesirable surface effect after relatively short periods of wear or washing. 10 In suiting materials, the pilling effect shows up mainly on collars, cuffs, sleeves and other portions of the garments that normally rub against each other or against other surfaces during wear of the garment, and as a result of this abrasion, even though slight, numerous pills or balls form on the surface. This undesirable effect is especially noticeable and pronounced in knitted wear, such as sweaters made of "Dacron." The numerous pills formed on the surface of the sweaters adhere so tenaciously that they cannot be removed by the usual brushing.

20 I have discovered, in accordance with the present invention, that this important commercial problem can be effectively solved by a heat treatment of these synthetic polyester fiber fabrics with a highly heated liquid. As a result of this heat treatment, the fabric shows little or no tendency to produce pills or balls even under severe abrasion.

25 In a commercially advantageous example of the process of my invention, I subject the polyester fiber fabric to an impregnation treatment with a highly heated, non-aqueous, non-evaporative liquid that quickly heats the polyester textile material to the temperature of the liquid and effects rapid penetration thereof by this liquid. In fact, the penetration is sufficiently deep and uniform that 30 a small amount of the treating liquid remains imbedded in the fibers of the fabric even after thorough washing and drying of the fabric. This small residual impregnant in the fabric aids in identifying the polyester textile material that has the non-pilling characteristic established 35 therein by treatment of the fabric at a high temperature with the highly heated liquid in accordance with the present invention, and also confers other desirable properties such as those of an internal lubricant which enables garment manufacturers more readily and conveniently to process these fabrics during the garment manufacturing operations. For example, in cutting to pattern numerous layers of stacked polyester fabrics that have been treated in accordance with the present invention, the residual impregnant greatly facilitates the cutting operation by helping to keep the cutting knife cool.

40 For carrying out the process of my invention, I have found that it is important to utilize as the highly heated liquid medium, a liquid having a high boiling point substantially above the boiling point of water, e.g. about 45 250° F. or higher, there being no upper limit on the boiling point which in practice may run as high as about 550° F. with certain high boiling liquids.

50 Another important characteristic of the liquid to be used in my process is that it should be non-evaporative, like glycerine and other polyhydric alcohols, as distinct from the evaporative or vaporizable lower aliphatic alcohols or ethers.

55 A further important aspect of the heated liquid medium used in my invention is that it should be anhydrous or free of water so as to maintain the desired high boiling point of the liquid medium and to avoid bubbling and evaporation of the liquid which would otherwise occur in the presence of water during the high temperature treatment.

70 Suitable, but non-limiting, examples of liquids for use in my invention are polyhydroxy compounds such as

ethylene glycol, diethylene glycol, propylene glycol, di-propylene glycol, butylene glycol and glycerine. Of the foregoing, the glycols and glycol ethers or polyglycols are preferred. In view of the fact that the effectiveness of the highly heated solvent apparently does not depend upon any of its chemical properties, but instead upon its physical properties, particularly the high boiling point and non-evaporative characteristics, the solvent may be selected from any material having these essential properties even though they differ substantially in chemical properties. From the standpoint of low cost, commercial availability and wide solvent properties, I have found diethylene glycol to be a preferred material. Its boiling point is approximately 430° F. Another preferred material is dipropylene glycol, boiling point approximately 450° F. These compounds have no adverse effects on the polyester textile materials, are water-soluble and are therefore easily removable or substantially removable from the polyester textile material after treatment. Due to its somewhat higher boiling point, and consequently lower vapor pressure at a given elevated temperature of treatment, the dipropylene glycol offers unusually attractive properties for commercial use.

These and similar non-aqueous, non-evaporative high boiling liquids will, when highly heated, penetrate and impregnate the polyester textile material to impart to it anti-pilling or other new and desirable properties and to facilitate subsequent additional treatment such as dyeing thereof. By using this highly heated liquid for conditioning the polyester textile material before application of the dyestuff, the fibers of the polyester textile material are made markedly receptive to penetration and impregnation by the dyestuff. When the polyester textile material is first conditioned in this manner, the subsequent dyeing operation can be carried out in a markedly shorter time than is normally required.

At the present time it is very difficult to dye polyester materials. Various types of high pressure equipment have been designed to increase the boiling point of water, thus causing the dyestuff to penetrate more readily into the polyester fibers. This pressure equipment is very costly and is by no means the answer to efficient dyeing procedures. Another method that has been proposed for increasing the dye absorption of the polyester material is dyeing on conventional equipment using carriers in the dyebath. The most effective carriers are phenolic compounds. These phenols have several disadvantages such as that they affect the light fastness adversely, are very difficult to remove from the polyester material, and increase the dyeing cost considerably. An illustration of the dyeing problems encountered when polyester materials are dyed by conventional methods is that one large textile concern currently has a fully pressurized dye plant under construction solely for the dyeing of polyester materials. The dyeing cycle for polyester materials on conventional equipment is approximately 8-14 hours, depending on the depth of shade desired.

The polyester material conditioned in accordance with the present invention may be dyed very readily on conventional dyeing equipment without the use of carriers or high pressure equipment. The full dyeing cycle is less than 3 hours and complete dyestuff exhaustion is achieved at comparatively low temperatures. It has been found that complete dye exhaustion takes place at temperatures as low as 180° F.

Another important characteristic of the heated organic liquid used in the process of the present invention is its solubility in water, whereby the superficially adhering organic liquid may be easily removed or substantially completely removed from the treated polyester textile material in a simple manner such as by washing with water, while still leaving a relatively small amount entrapped in the fiber structure.

Further, the liquid heating medium should preferably be neutral in character, neither strongly acid nor strongly basic, and otherwise substantially inert to the polyester textile material to avoid any adverse effects when the polyester textile material is impregnated with the hot liquid.

Regarding the form of polyester textile material that may be treated in accordance with the process of my invention, this process has been found to be applicable to practically any and all forms, such as filaments, staple fibers, threads, yarns and woven or knitted goods.

The optimum operating temperature for heat treatment of the fabric or other polyester textile material will vary with the particular fiber, and particularly its resistance to heat. For example, when treating "Dacron" in the form of fabrics, the temperature should not go substantially above 365° F. with one kind of "Dacron," namely "Dacron" type 64, although with another type of "Dacron," namely type 54, a temperature of about 385° F. is advantageously employed. In general, the organic liquids used should have a boiling point within the range of about 250° F. to 550° F., and preferably about 350° to 550° F.; should not harm the fabric or other polyester material; and should be removable or substantially removable therefrom after the heat treatment has been completed.

Where it is desired to effect dyeing subsequently to the wet heat treating process of this invention, practically any and all known types of dyestuffs suitable for the textile materials undergoing treatment may be used. These include vats, Indigosols, basic dyes, acid dyes and dispersed dyes, as well as dyestuffs more recently developed for dyeing some of the newer synthetic fibers, such as, for example, "Latyl" dyes, which are also dispersed dyes.

Regarding the equipment necessary for carrying out this new polyester textile material conditioning method, it is not critical in character and is subject to wide variations. The essential requirements are a suitable container for heating the non-aqueous, non-evaporative liquid treating agent to the desired higher temperatures.

The following are illustrative but non-limiting examples of the process of my invention, in which synthetic polyester fiber textile materials are treated at high temperatures to prevent or minimize pilling effects and to impart thereto other improved properties such as better dye receptivity.

#### Example 1

A clean, dry, "Dacron" fabric is passed through a bath of diethylene glycol heated to a temperature of approximately 360-365° F. I have found that the effectiveness of this treatment can be obtained almost immediately, that is, with about ten seconds' treatment of the cloth in this highly heated diethylene glycol bath. After the "Dacron" fabric passes through this liquid bath, the surplus diethylene glycol is squeezed off by squeeze rolls or the like and the treated cloth is then passed through a water bath at ordinary room temperature which removes substantially all of the diethylene glycol but leaves a very small amount of the diethylene glycol entrapped in the "Dacron" fibers. After washing with water, the polyester fabric is dried and may be used as such or it may be dyed or otherwise finished as desired. If it is to be dyed immediately following the conditioning step, then of course it need not first be dried.

In the event other similar non-aqueous, non-evaporative, water-soluble liquids such as those mentioned above are used for effecting the conditioning treatment, then the procedure described in Example 1 above would be generally followed with any necessary adjustments of the temperature for the specific treating liquid, although in general the temperatures would be of the same high order and sufficient to effect at least a partial penetration of the polyester textile fiber fabric with the highly heated

treating liquid, as a result of which the fabric will not thereafter show the usual pilling effect upon abrasion.

Generally speaking, the residual treating liquid retained in and carried by the polyester textile material, even after washing and drying, will be relatively small such as of the order of about 2% by weight.

It has been found that the process of my invention may be applied satisfactorily, as above described, to cloth or the like consisting of a single type of "Dacron" polyester fibers, or composed of a mixture of "Dacron" and other fabrics, such as, for example, "Dacron" and wool, etc., and a subsequent uniform or "union" dyeing result obtained, assuming of course the proper selection of dyestuff or dyestuffs suited for dyeing the respective fibers.

*Example 2*

A number of skeins of "Dacron" polyester tow were treated as follows: skeins Nos. 1, 2 and 3 were "Dacron" type 54 and one-half of each skein was immersed for 15 seconds in dipropylene glycol at a temperature of 385° F. Skeins Nos. 4 and 5 were "Dacron" type 64 and one-half of each skein was treated for 15 seconds in dipropylene glycol at a temperature of 365° F., it being possible to treat the type 64 product at a somewhat lower temperature.

After treating the "Dacron" skeins in dipropylene glycol in the foregoing fashion, the treated skeins were chilled in cold water for the purpose of suddenly closing the fiber pores and thereby entrapping relatively small traces of dipropylene glycol in the fiber. The skeins were then washed in warm water and subjected to dyeing in an otherwise conventional manner without the use of carrier or high pressure equipment, i.e., in substantially the same manner as in the conventional dyeing of acetate-rayon. In each case the dyestuff was pasted with a small amount of Alkanol HCS (du Pont) which acts as a dispersing agent for the dyestuff.

All dyeings were carried out in an aqueous medium at a temperature of 200° F. for a period of one-half hour. The dyestuffs employed were as follows:

Skein No. 1—Acetamine Rubine B (du Pont)

Skein No. 2—Eastman Blue BNN (Tennessee-Eastman)

Skein No. 3—Acetamine Fast Yellow 4 RL (du Pont)

Skein No. 4—Latyl Brilliant Blue 2G (du Pont)

Skein No. 5—Sevron Blue 5G (du Pont)

The first four dyestuffs are dispersed dyestuffs, while the last dyestuff is a cationic dyestuff.

In all cases the conditioned "Dacron" (i.e., the half of the skein that had been immersed in the heated dipropylene glycol) dyed darker and more evenly than non-conditioned "Dacron."

The process as described in the specification and defined in the claims herein for quickly heating the polyester textile material of the kind indicated above with an anhydrous organic liquid at a temperature between approximately 250° and 550° F., but preferably between about 350° and 550° F., but below the softening or damaging point for the polyester textile material, requires a relatively very short time, e.g. less than about one minute and usually in the order of eight to fifteen seconds time as specified in the illustrative but non-limiting examples herein.

This application is a continuation-in-part of my prior application Serial No. 491,173, filed February 28, 1955, now abandoned, which in turn is a continuation-in-part of my prior application Serial No. 415,155, filed March 9, 1954, now abandoned.

The above described materials, conditions and pro-

cedures are subject to modifications and variations, as indicated in the appended claims.

What is claimed is:

1. A process of improving the dyeability and minimizing the pilling effects in a synthetic polyester textile material comprising a condensation polymer of terephthalic acid and ethylene glycol, comprising the steps of immersing the textile material in a heated, anhydrous, relatively high-boiling, water-soluble, inert, organic liquid medium in the substantial absence of any dyestuff and at an elevated temperature of at least 250° F. but below the softening point of the textile material, for a period of time sufficient to effect impregnation of the textile material with the heated organic liquid medium and to modify the fiber structure of the textile material by penetration of said organic liquid medium into said fiber structure but without otherwise affecting the fiber structure, removing the textile material from the heated organic liquid medium, and immediately thereafter contacting the textile material with relatively cool water, thereby substantially removing the adhering organic liquid medium from the textile material while leaving entrapped within the fiber structure thereof a small residual amount of said organic liquid medium.
2. A process as defined in claim 1 in which the organic liquid medium is at an elevated temperature of at least 350° F.
3. A product as prepared by the process of claim 1.
4. A process of improving the dyeability and minimizing the pilling effects in a synthetic polyester textile material comprising a condensation polymer of terephthalic acid and ethylene glycol, comprising the steps of immersing the textile material in a heated, anhydrous, relatively high-boiling, water-soluble, inert, organic liquid medium consisting essentially of a polyhydric alcohol selected from the group consisting of ethylene glycol, diethylene glycol, propylene glycol, dipropylene glycol, butylene glycol, and glycerine in the substantial absence of any dyestuff, which liquid medium is at an elevated temperature of at least 250° F. but below the softening point of the textile material, for a period of time sufficient to effect impregnation of the textile material with the heated organic liquid medium and to modify the fiber structure of the textile material by penetration of said organic liquid medium into said fiber structure but without otherwise affecting the fiber structure, removing the textile material from the heated organic liquid medium, and immediately thereafter contacting the textile material with relatively cool water, thereby substantially removing the adhering organic liquid medium from the textile material while leaving entrapped within the fiber structure thereof a small residual amount of said organic liquid medium.
5. A process as defined in claim 4 in which the organic liquid medium is at an elevated temperature of at least 350° F.

References Cited in the file of this patent

UNITED STATES PATENTS

- |           |                    |               |
|-----------|--------------------|---------------|
| 2,461,612 | Olpin et al. ----- | Feb. 15, 1949 |
| 2,537,177 | Woodruff -----     | Jan. 8, 1951  |
| 2,663,612 | Gibson -----       | Dec. 22, 1953 |

FOREIGN PATENTS

- |         |                   |               |
|---------|-------------------|---------------|
| 230,891 | Switzerland ----- | Feb. 15, 1944 |
|---------|-------------------|---------------|

OTHER REFERENCES

- American Dyestuff Reporter, Nov. 13, 1950, page 790.  
Du Pont Bulletin CSB-D-35, Dacron, July 1954, pages 1, 2 and 3.